



US006113825A

# United States Patent [19]

Chuah

[11] Patent Number: 6,113,825

[45] Date of Patent: Sep. 5, 2000

[54] **PROCESS FOR PREPARING POLY(TRIMETHYLENE TEREPHTHALATE) CARPET YARN**

[75] Inventor: **Hoe Hin Chuah**, Houston, Tex.

[73] Assignee: **Shell Oil Company**, Houston, Tex.

[21] Appl. No.: **08/969,726**

[22] Filed: **Nov. 13, 1997**

## Related U.S. Application Data

[63] Continuation of application No. 08/538,695, Oct. 3, 1995, abandoned, which is a continuation-in-part of application No. 08/435,065, May 8, 1995, abandoned.

[51] **Int. Cl.<sup>7</sup>** ..... **D01D 5/16**; D01F 6/62; D02G 3/02

[52] **U.S. Cl.** ..... **264/103**; 28/271; 264/210.7; 264/210.8; 264/211.12; 264/211.14

[58] **Field of Search** ..... 264/103, 210.7, 264/210.8, 211.12, 211.14; 28/271

## References Cited

### U.S. PATENT DOCUMENTS

3,998,042 12/1976 Reese ..... 57/245

4,195,052 3/1980 Davis et al. ..... 264/210.5  
4,877,572 10/1989 Clarke et al. ..... 264/555  
5,645,782 7/1997 Howell et al. ..... 264/103  
5,662,980 9/1997 Howell et al. ..... 428/88

Primary Examiner—Leo B. Tentoni

## ABSTRACT

Poly(trimethylene terephthalate) is formed into a bulk continuous filament yarn by melt-spinning poly(trimethylene terephthalate) at a temperature of 240 to 280° C. to produce a plurality of spun filaments, cooling the spun filaments, converging the spun filaments into a yarn, drawing the yarn at a first draw ratio of 1.01 to about 2 in a first drawing stage defined by at least one feed roller and at least one first draw roller wherein at least one feed roller is operated at less than 100° C. and each of the draw rollers is heated to a temperature greater than that of the feed roller and between 50 and 150° C., subsequently drawing the yarn at a second draw ratio of at least about 2.2 times that of the first draw ratio in the second drawing stage defined by at least one first draw roller and at least one second draw roller, wherein at least one second draw roller is heated to a temperature greater than that of the first draw roller and within the range of 100 to 200° C., and texturing the drawn yarn and cooling the textured filaments.

13 Claims, 1 Drawing Sheet





FIG. 1



FIG. 2

**PROCESS FOR PREPARING  
POLY(TRIMETHYLENE TEREPHTHALATE)  
CARPET YARN**

**CROSS-REFERENCE TO RELATED  
APPLICATION**

This is a continuation of application Ser. No. 08/538,695, filed Oct. 3, 1995, now abandoned, which is a continuation-in-part of application Ser. No. 08/435,065, filed May 8, 10 1995, now abandoned.

**BACKGROUND OF THE INVENTION**

This invention relates to the spinning of synthetic polymeric yarns. In a specific embodiment, the invention relates to spinning poly(trimethylene terephthalate) into yarn suitable for carpets.

Polyesters prepared by condensation polymerization of the reaction product of a diol with a dicarboxylic acid can be spun into yarn suitable for carpet fabric. U.S. Pat. No. 3,998,042 describes a process for preparing poly(ethylene terephthalate) yarn in which the extruded fiber is drawn at high temperature (160° C.) with a steam jet assist, or at a lower temperature (95° C.) with a hot water assist. Poly (ethylene terephthalate) can be spun into bulk continuous filament (BCF) yarn in a two-stage drawing process in which the first stage draw is at a significantly higher draw ratio than the second stage draw. U.S. Pat. No. 4,877,572 describes a process for preparing poly(butylene terephthalate) BCF yarn in which the extruded fiber is drawn in one stage, the feed roller being heated to a temperature 30° C. above or below the Tg of the polymer and the draw roller being at least 100° C. higher than the feed roll. The application of conventional polyester spinning processes to prepare poly(trimethylene terephthalate) BCF results in yarn which is of low quality and poor consistency. It would be desirable to have a process for preparing high-quality BCF carpet yarn from poly(trimethylene terephthalate).

It is therefore an object of the invention to provide a process for preparing high-quality bulk continuous filament yarn from poly(trimethylene terephthalate).

**SUMMARY OF THE INVENTION**

According to the invention, poly(trimethylene terephthalate) is formed into a bulk continuous filament yarn by a process comprising:

- (a) melt-spinning poly(trimethylene terephthalate) at a temperature within the range of about 240° to about 280° C. to produce a plurality of spun filaments;
- (b) cooling the spun filaments;
- (c) converging the spun filaments into a yarn;
- (d) drawing the yarn at a first draw ratio within the range of about 1.01 to about 2 in a first drawing stage defined by at least one feed roller and at least one first draw roller, each of said at least one feed roller operated at a temperature less than about 100° C. and each of said at least one draw roller heated to a temperature greater than the temperature of said at least one feed roller and within the range of about 50 to about 150° C.;
- (e) subsequently drawing the yarn at a second draw ratio of at least about 2.2 times that of the first draw ratio in a second drawing stage defined by said at least one first draw roller and at least one second draw roller, each of said at least one second draw roller heated to a temperature greater than said at least one first draw roller and within the range of about 100 to about 200° C.; and
- (f) winding the drawn yarn.

The process may optionally include texturing the drawn yarn prior to or after winding step (f).

The process of the invention permits the production of poly(trimethylene terephthalate) bulk continuous filament 5 yarn suitable for high-quality carpet.

**BRIEF DESCRIPTION OF THE FIGURES**

FIG. 1 is a schematic diagram of one embodiment of the invention yarn preparation process.

10 FIG. 2 is a schematic diagram of a second embodiment of the invention process.

**DETAILED DESCRIPTION OF THE  
INVENTION**

The fiber-spinning process is designed specifically for poly(trimethylene terephthalate), the product of the condensation polymerization of the reaction product of trimethylene diol (also called "1,3-propane diol") and a terephthalic acid or an ester thereof, such as terephthalic acid and dimethyl terephthalate. The poly(trimethylene terephthalate) may be derived from minor amounts of other monomers such as ethane diol and butane diol as well as minor amounts of other diacids or diesters such as isophthalic acid. Poly (trimethylene terephthalate) having an intrinsic viscosity (i.v.) within the range of about 0.8 to about 1.0 dl/g, preferably about 0.86 to about 0.96 dl/g (as measured in a 50/50 mixture of methylene chloride and trifluoroacetic acid at 30° C.) and a melting point within the range of about 215 to about 230° C. is particularly suitable. The moisture content of the poly(trimethylene terephthalate) should be less than about 0.005% prior to extrusion. Such a moisture level can be achieved by, for example, drying polymer pellets in a dryer at 150–180° C. until the desired dryness has been achieved.

One embodiment of the invention process can be described by reference to FIG. 1. Molten poly(trimethylene terephthalate) which has been extruded through a spinneret into a plurality of continuous filaments 1 at a temperature within the range of about 240 to about 280° C., preferably about 250 to about 270° C., and then cooled rapidly, preferably by contact with cold air, is converged into a multifilament yarn and the yarn is passed in contact with a spin finish applicator, shown here as kiss roll 2. Yarn 3 is passed around denier control rolls 4 and 5 and then to a first drawing stage defined by feed roll 7 and draw roll 9. Between rolls 7 and 9, yarn 8 is drawn at a relatively low draw ratio, within the range of about 1.01 to about 2, preferably about 1.01 to about 1.35. Roller 7 is maintained at a temperature less than about 100° C., preferably within the range of about 40 to about 85° C. Roller 7 can be an unheated roll, in which case its temperature of operation will be somewhat elevated (30–45° C.) due to friction and the temperature of the spun fiber. Roller 9 is maintained at a temperature within the range of about 50 to about 150° C., preferably about 90 to about 140° C.

Drawing speeds of greater than 1000 m/min. are possible with the invention process, with drawing speeds greater than 1800 m/min. desirable because of the high tenacity of the 40 resulting yarn.

Drawn yarn 10 is passed to a second drawing stage, defined by draw rolls 9 and 11. The second-stage draw is carried out at a relatively high draw ratio with respect to the first-stage draw ratio, generally at least about 2.2 times that of the first stage draw ratio, preferably at a draw ratio within the range of about 2.2 to about 3.4 times that of the first stage. Roller 11 is maintained at a temperature within the 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130

range of about 100 to about 200° C. In general, the three rollers will be sequentially higher in temperature. The selected temperature will depend upon other process variables, such as whether the BCF is made with separate drawing and texturing steps or in a continuous draw/texturing process, the effective heat transfer of the rolls used, residence time on the roll, and whether there is a second heated roll upstream of the texturing jet. Drawn fiber 12 is passed in contact with optional relax roller 13 for stabilization of the drawn yarn. Stabilized yarn 14 is passed to optional winder 15 or is sent directly to the texturing process.

The drawn yarn is bulked by suitable means such as a hot air texturing jet. The preferred feed roll temperature for texturing is within the range of about 150 to about 220° C. The texturing air jet temperature is generally within the range of about 150 to about 210° C., and the texturing jet pressure is generally within the range of about 50 to about 120 psi to provide a high-bulk BCF yarn. Wet or superheated steam can be substituted for hot air as the bulking medium.

FIG. 2 shows a second embodiment of the two-stage drawing process showing texturing steps downstream of the drawing zone. Molten poly(trimethylene terephthalate) is extruded through spinneret 21 into a plurality of continuous filaments 22 and is then quenched by, for example, contact with cold air. The filaments are converged into yarn 24 to which spin finish is applied at 23. Yarn 27 is advanced to the two-stage draw zone via rolls 25 and 26, which may be heated or non-heated.

In the first draw stage, yarn 31 is drawn between feed roll 28 and draw roll 29 at a draw ratio within the range of about 1.01 and about 2. Drawn yarn 32 is then subjected to a second draw at a draw ratio at least about 2.2 times the first draw ratio, preferably a draw ratio within the range of about 2.2 to about 3.4 times that of the first draw. The temperature of roll 28 is less than about 100° C. The temperature of draw roll 29 is within the range of about 50 to about 150° C. The temperature of draw roll 30 is within the range of about 100 to about 200° C. Drawn yarn 33 is advanced to heated rolls 34 and 35 to preheat the yarn for texturing. Yarn 36 is passed through texturing air jet 37 for bulk enhancement and then to jet screen cooling drum 38. Textured yarn 39 is passed through tension control 40, 41 and 42 and then via idler 43 to optional entangler 44 for yarn entanglement if desired for better processing downstream. Entangled yarn 45 is then advanced via idler 46 to an optional spin finish applicator 47 and is then wound onto winder 48. The yarn can then be processed by twisting, texturing and heat-setting as desired and tufted into carpet as is known in the art of synthetic carpet manufacture.

Poly(trimethylene terephthalate) yarn prepared by the invention process has high bulk (generally within the range of about 20 to about 45%, preferably within the range of about 26 to about 35%), resilience and elastic recovery, and is useful in the manufacture of carpet, including cut-pile, loop-pile and combination-type carpets, mats and rugs. Poly(trimethylene terephthalate) carpet has been found to exhibit good resiliency, stain resistance and dyability with disperse dyes at atmospheric boil with optional carrier.

#### EXAMPLE 1

##### Effect of Intrinsic Viscosity on Poly(trimethylene terephthalate) Fiber Drawing

Four poly(trimethylene terephthalate) polymers having intrinsic viscosities of 0.69, 0.76, 0.84 and 0.88 dl/g, respectively, were each spun into 70 filaments with trilobal cross-sections using a spinning machine having a take-up

and drawing configuration as shown in FIG. 1. Roll 1 (see detail below) was a double denier control roll; roll 2 ran at a slightly higher speed to maintain a tension and act as a feed roll for drawing. First stage drawing took place between rolls 2 and 3, and second-stage drawing took place between rolls 3 and 4. The drawn yarn contacted relax roll 5 prior to wind-up. The spin finish was a 15% Lurol PF 4358-15 solution from G. A. Gouston Company applied with a kiss roll.

Fiber extrusion and drawing conditions for each polymer were as follows:

| Extrusion Conditions      |        |            |            |
|---------------------------|--------|------------|------------|
|                           | Units  |            |            |
| Polymer IV (dl/g):        |        | 0.84, 0.88 | 0.69, 0.76 |
| Extruder Temp. Profile:   |        |            |            |
| Zone 1                    | ° C.   | 230        | 225        |
| Zone 2                    | ° C.   | 250        | 235        |
| Zone 3                    | ° C.   | 250        | 235        |
| Zone 4                    | ° C.   | 250        | 235        |
| Melt Temp.                | ° C.   | 255        | 240        |
| Extrusion Pack Pressure   | psi    | 1820-2820  | 500-1300   |
| Denier Control Roll Speed | m/min. | 225        | 220        |

| Fiber Drawing Conditions |                   |      |      |      |      |
|--------------------------|-------------------|------|------|------|------|
|                          | Polymer IV (dl/g) | 0.88 | 0.84 | 0.76 | 0.69 |
| Roll Temp.: ° C.         |                   |      |      |      |      |
| Roll 2                   |                   | 80   | 80   | 80   | 80   |
| Roll 3                   |                   | 95   | 95   | 95   | 95   |
| Roll 4                   |                   | 155  | 155  | 155  | 155  |
| Roll 5                   |                   | RT   | RT   | RT   | RT   |
| Roll Speeds: m/min.      |                   |      |      |      |      |
| Roll 2                   |                   | 230  | 230  | 230  | 230  |
| Roll 3                   |                   | 310  | 310  | 404  | 404  |
| Roll 4                   |                   | 1020 | 1165 | 1089 | 1089 |
| Roll 5                   |                   | 1035 | 1102 | 1075 | 1075 |
| First Stage Draw Ratio   |                   | 1.35 | 1.35 | 1.76 | 1.76 |
| Second Stage Draw Ratio  |                   | 3.29 | 3.29 | 2.70 | 2.70 |

TABLE 1

| Run | I.V. (dl/g) | Yarn Count (den.) | Tenacity (g/den.) | % Elongation |
|-----|-------------|-------------------|-------------------|--------------|
| 1   | 0.69        | 1182              | 1.51              | 70.7         |
| 2   | 0.76        | 1146              | 1.59              | 79.7         |
| 3   | 0.84        | 1167              | 2.03              | 89.0         |
| 4   | 0.88        | 1198              | 2.24              | 67.5         |

Poly(trimethylene terephthalate) of intrinsic viscosities 0.69 and 0.76 (Runs 1 and 2) gave yarn of inferior tensile properties compared with the yarn of Runs 3 and 4. These polymers were re-spun at a lower extruder temperature profile. Although they could be spun and drawn, the fibers had high die swell. When the fiber cross-sections were examined with an optical microscope, the 0.69 i.v. fibers swelled to a point that they were no longer trilobal in shape and resembled delta cross-sections. They also had relatively low tenacity.

#### EXAMPLE 2

##### Two-Stage Drawing of PTT Fibers

0.88 i.v. poly(trimethylene terephthalate) was extruded into 72 filaments having trilobal cross-section using a fiber-

spinning machine having take-up and drawing configurations as in Example 1. Spin finish was applied as in Example 1. Extrusion and drawing conditions were as follows.

| Extrusion Conditions          |        | Drawing Conditions |                   |               |
|-------------------------------|--------|--------------------|-------------------|---------------|
| Extruder Temperature Profile: | Units  | Rolls              | Temperature, ° C. | Speed, m/min. |
| Zone 1                        | ° C.   | 230                |                   |               |
| Zone 2                        | ° C.   | 260                |                   |               |
| Zone 3                        | ° C.   | 260                |                   |               |
| Zone 4                        | ° C.   | 260                |                   |               |
| Melt Temp.                    | ° C.   | 265                |                   |               |
| Denier Control Roll Speed     | m/min. | 230                |                   |               |

and texturizer air jet temperatures were kept constant, and the air jet pressure was varied from 50 to 100 psi to prepare poly(trimethylene terephthalate) BCF of various bulk levels.

Drawing and texturing conditions were as follows.

5

| Fiber Drawing Conditions |            |          |          |          |          |          |         |
|--------------------------|------------|----------|----------|----------|----------|----------|---------|
| Units                    | Runs       |          |          |          |          |          |         |
|                          | 5          | 6        | 7        | 8        | 9        | 10       | 11      |
| Roll 2 Temp./Speed       | ° C./m/min | 80/235   | 80/235   | 100/235  | 100/235  | 100/235  | 100/235 |
| Roll 3 Temp./Speed       | ° C./m/min | 90/317   | 100/286  | 100/817  | 100/817  | 100/993  | 100/945 |
| Roll 4 Temp./Speed       | ° C./m/min | 155/1123 | 100/1021 | 155/1047 | 140/1103 | 130/1044 | 140/996 |
| Roll 5 Temp./Speed       | ° C./m/min | RT/1096  | RT/1011  | RT/1029  | RT/1082  | RT/1134  | RT/1019 |
| 1st Stage Draw Ratio     |            | 1.35     | 1.22     | 3.48     | 3.48     | 4.23     | 4.02    |
| 2nd Stage Draw Ratio     |            | 3.55     | 3.57     | 1.28     | 1.35     | 1.05     | 1.05    |
| Total Draw Ratio         |            | 4.79     | 4.36     | 4.45     | 4.70     | 4.87     | 4.44    |
| Yarn Count, den.         | den.       | 1225     | 1281     | 1275     | 1185     | 1210     | 1288    |
| Tenacity, g/den.         | g/den.     | 1.95     | 1.95     | 1.61     | 1.32     | 1.85     | 1.11    |
| Elongation               | %          | 55       | 75       | 70       | 76       | 78       | 86      |

It was observed during spinning and drawing that, when the first-stage draw ratio (between rolls 2 and 3) was less than about 1.5, as in Runs 5 and 6, there were fewer broken filaments and the tenacities of the filaments were generally higher than when first-stage draw was higher than about 1.5. When the first-stage draw was increased to greater than 3 (Runs 7, 8, 9, 10, and 11), it was observed that the fibers had a white streaky appearance, the threadlines were loopy, and there were frequent filament wraps on the draw rolls. The process was frequently interrupted with fiber breaks.

### EXAMPLE 3

Spinning, Drawing and Texturing Poly(trimethylene terephthalate) BCF to High Bulk.

The extrusion conditions in this experiment were the same as in Example 2. The fibers were spun, drawn and wound as in Example 1. They were then textured by heating the fibers on a feed roll and exposing the fibers to a hot air jet. The textured fibers were collected as a continuous plug on a jet-screen cooling drum. Partial vacuum was applied to the drum to pull the ambient air to cool the yarns and keep them on the drum until they were wound. The yarns were air entangled between the drum and the winder. The feed roll

35

40

45

50

55

Yarn bulk and shrinkage were measured by taking 18 wraps of the textured yarn in a denier creel and tying it into a skein. The initial length  $L_0$  of the skein was 22.1 inches in English unit creel. A 1 g weight was attached to the skein and it was hung in a hot-air oven at 130° C. for 5 minutes. The skein was removed and allowed to cool for 3 minutes. A 50 g weight was then attached and the length  $L_1$  was measured after 30 seconds. The 50 g weight was removed, a 10 Lb weight was attached, and the length  $L_2$  was measured after 30 seconds. Percent bulk was calculated as  $(L_0 - L_1)/L_0 \times 100\%$  and shrinkage was calculated as  $(L_0 - L_2)/L_0 \times 100\%$ . Results are shown in Table 2.

| TABLE 2     |                  |        |             |
|-------------|------------------|--------|-------------|
| Package No. | Yarn Count, den. | % Bulk | % Shrinkage |
| T50         | 1437             | 32.6   | 3.6         |
| T60         | 1406             | 35.7   | 2.7         |
| T70         | 1455             | 39.4   | 3.2         |
| T80         | 1500             | 38.0   | 3.6         |
| T90         | 1525             | 37.6   | 4.1         |
| T100        | 1507             | 38.0   | 3.6         |

The experiment showed that poly(trimethylene terephthalate) BCF can be textured to high bulk with a hot air texturizer.

## EXAMPLE 4

## Carpet Resiliency Comparison

Poly(trimethylene terephthalate) BCF yarns were made in two separate steps: (1) spinning and drawing set-up as in Example 1 and (2) texturing. Extrusion, drawing and texturing conditions for the poly(trimethylene terephthalate) yarns were as follows.

| Extrusion Conditions |       |      |
|----------------------|-------|------|
| Extruder Temperature | Units |      |
| Zone 1               | ° C.  | 240  |
| Zone 2               | ° C.  | 255  |
| Zone 3               | ° C.  | 255  |
| Zone 4               | ° C.  | 255  |
| Melt Temperature     | ° C.  | 260  |
| Pack Pressure        | psi   | 1830 |

  

| Drawing Conditions |             |          |
|--------------------|-------------|----------|
|                    | Units       |          |
| Roll 1 Temp.       | ° C./m/min. | RT/223   |
| Roll 2 Temp.       | ° C./m/min. | 80/230   |
| Roll 3 Temp.       | ° C./m/min. | 95/288   |
| Roll 4 Temp.       | ° C./m/min. | 150/1088 |
| Roll 5 Temp.       | ° C./m/min. | RT/1000  |

  

| Texturing Conditions |        |     |
|----------------------|--------|-----|
|                      | Units  |     |
| Feed Roll Temp.      | ° C.   | 180 |
| Feed Roll Speed      | m/min. | 980 |
| Air Jet Temp.        | ° C.   | 180 |
| Air Jet Pressure     | psi    | 90  |
| Interlacing Pressure | psi    | 10  |

The yarn produced was 1150 denier with 2.55 g/den tenacity and 63% elongation. The textured yarn was twisted, heat set as indicated, and tufted into carpets. Performances of the poly(trimethylene terephthalate) carpets were compared with a commercial 1100 denier nylon 66 yarn. Results are shown in Table 3.

TABLE 3

| Run                                  | Twist/<br>Inch | Heat<br>Setting<br>Conditions | Accelerated<br>Floor<br>Traffic<br>Rating | % Loss<br>in Pile<br>Thick-<br>ness |
|--------------------------------------|----------------|-------------------------------|-------------------------------------------|-------------------------------------|
| 12 (Poly(trimethylene terephthalate) | 4.5 x 4.5      | 270° F.<br>Autoclave          | 3.75                                      | 2.4                                 |
| 13 (Poly(trimethylene terephthalate) | 4.5 x 4.5      | 180° C.<br>Seussen            | 3.5                                       | 7.1                                 |
| 14 (Poly(trimethylene terephthalate) | 5.0 x 5.0      | 270° F.<br>Autoclave          | 3.75                                      | 1.7                                 |
| 15 nylon 66                          | 4.0 x 4.0      | 270° F.<br>Autoclave          | 3.0                                       | 6.4                                 |
| 16 nylon 66                          | 4.0 x 4.0      | 190° C.<br>Seussen            | 3.5                                       | 4.5                                 |

The heat-set yarns were tufted into 24 oz. cut-pile Saxony carpets in  $\frac{1}{8}$ " gauge,  $\frac{1}{16}$ " pile height, and dyed with disperse

blue 56 (without a carrier) at atmospheric boil into medium blue color carpets. Visual inspection of the finished carpets disclosed that the poly(trimethylene terephthalate) carpets (Runs 12, 13 and 14) had high bulk and excellent coverage which were equal to or better than the nylon controls (Runs 15 and 16). Carpet resiliency was tested in accelerated floor trafficking with 20,000 footsteps. The appearance retention was rated 1 (severe change in appearance), 2 (significant change), 3 (moderate change), 4 (slight change) and 5 (no change). As can be seen in Table 3, the poly(trimethylene terephthalate) carpets were equal to or better than the nylon 66 controls in the accelerated walk tests and in percent thickness loss.

## EXAMPLE 5

One-Step Processing of Poly(trimethylene terephthalate) BCF Yarn from Spinning to Texturing

25 Poly(trimethylene terephthalate) (i.v. 0.90) was extruded into 72 trilobal cross-section filaments. The filaments were processed on a line as shown in FIG. 2 having two cold rolls, three draw rolls and double yarn feed rolls prior to texturing. The yarns were textured with hot air, cooled in a rotating jet screen drum and wound up with a winder. Lurol NF 3278 CS (G. A. Goulston Co.) was used as the spin finish. Texturing conditions were varied to make poly(trimethylene terephthalate) BCF yarns having different bulk levels. 30 35 Extrusion, drawing, texturing and winding conditions were as follows.

| Extrusion Conditions          |       |      |
|-------------------------------|-------|------|
| Extruder Temperature Profiles | Units |      |
| Zone 1                        | ° C.  | 240  |
| Zone 2                        | ° C.  | 260  |
| Zone 3                        | ° C.  | 260  |
| Zone 4                        | ° C.  | 265  |
| Melt Temperature              | ° C.  | 265  |
| Pump Pressure                 | psi   | 3650 |

  

| Drawing Conditions |               |      |
|--------------------|---------------|------|
| Temperature ° C.   | Speed, m/min. |      |
| Cold Roll 1        | RT            | 211  |
| Cold Roll 2        | RT            | 264  |
| Draw Roll 1        | 50            | 290  |
| Draw Roll 2        | 90            | 330  |
| Draw Roll 3        | 110           | 1100 |

65 The yarns were twisted, heat set and tufted into carpets for performance evaluation. Results are shown in Table 4.

TABLE 4

| Sample Number | Feed Roll Temp., °C. | Texturizing Jet Temp., °C. | Texturizing Jet Press., psi | Yarn Count, den. | % Bulk | % Shrinkage | Accelerated Walk Test Rating |
|---------------|----------------------|----------------------------|-----------------------------|------------------|--------|-------------|------------------------------|
| 1             | 150                  | 180                        | 70                          | 1490             | 19.2   | 1.58        | 3.25                         |
| 2             | 150                  | 180                        | 110                         | 1420             | 26     | 1.59        | 3.5                          |
| 3             | 150                  | 200                        | 110                         | 1546             | 30.5   | 1.59        | 3.0                          |
| 4             | 180                  | 180                        | 70                          | 1429             | 24.6   | 2.04        | 3.0                          |
| 5             | 180                  | 180                        | 110                         | 1496             | 29.8   | 1.81        | 3.5                          |
| 6             | 180                  | 200                        | 70                          | 1475             | 26.5   | 1.36        | 2.75                         |
| 7             | 180                  | 200                        | 110                         | 1554             | 32.8   | 0.86        | 3.0                          |
| 8             | 150                  | 190                        | 90                          | 1482             | 26     | 2.31        | 3.25                         |
| 9             | 180                  | 190                        | 90                          | 1430             | 29     | 1.58        | 3.5                          |
| 10            | 165                  | 190                        | 90                          | 1553             | 29     | 2.26        | 3.75                         |
| Nylon 6       |                      |                            |                             |                  |        |             | 3.5                          |
| Nylon 66      |                      |                            |                             |                  |        |             | 3.5                          |

## EXAMPLE 6

Effects of Draw Ratio and Roll Temperature on Yarn Properties

Poly(trimethylene terephthalate) (0.90 i.v.) was spun into 72 filaments with trilobal cross-sections using a machine as

texturing configuration similar to that shown in FIG. 1, with the yarn passing via unheated haul-off Roll 1, first-stage draw between Roll 1 and draw Roll 2, and second-stage draw between Roll 2 and dual Roll 3. The drawn yarns were then textured, relaxed and wound up. Extrusion conditions were as follows.

TABLE 5

| Sample:                | 1      | 2    | 3    | 4    | 5    | nylon 6 | nylon 66 |
|------------------------|--------|------|------|------|------|---------|----------|
| Roll 1 Temp.           | °C.    | 50   | 50   | 50   | 50   | 50      | 50       |
| Roll 2 Temp.           | °C.    | 90   | 90   | 90   | 90   | 90      | 90       |
| Roll 3 Temp.           | °C.    | 110  | 110  | 110  | 150  | 150     |          |
| Roll 1 Speed           | m/min. | 290  | 290  | 290  | 290  | 290     |          |
| Roll 2 Speed           | m/min. | 330  | 330  | 330  | 330  | 330     |          |
| Roll 3 Speed           | m/min. | 1000 | 1100 | 1150 | 1100 | 1000    |          |
| Draw Ratio             |        | 3.45 | 3.79 | 3.97 | 3.97 | 3.45    |          |
| Feed Roll Temp.        | °C.    | 165  | 165  | 165  | 165  | 165     |          |
| Feed Roll speed        | m/min. | 1000 | 1100 | 1150 | 1100 | 1000    |          |
| Texturing Jet Temp.    | °C.    | 190  | 190  | 190  | 190  | 190     |          |
| Texturing Jet Pressure | psi    | 90   | 90   | 90   | 90   | 90      |          |
| Interlacing Pressure   | psi    | 30   | 30   | 30   | 30   | 30      |          |
| Bulk                   | %      | 26.1 | 31.6 | 31.9 | 35.8 | 33      |          |
| Shrinkage              | %      | 1.75 | 2.04 | 2.13 | 2.26 | 1.92    |          |
| Walk Test Rating       |        | 4.0  | 3.5  | 3.5  | 3.5  | 3.5     | 3.5      |

described in Example 5. Extrusion conditions were as follows.

45

| Extrusion Conditions          |       | Extrusion Conditions    |         |         |
|-------------------------------|-------|-------------------------|---------|---------|
| Extruder Temperature Profiles | Units | Extruder Temp. Profiles | Trial 1 | Trial 2 |
| Zone 1                        | °C.   | Zone 1                  | 230° C. | 230     |
| Zone 2                        | °C.   | Zone 2                  | 260     | 245     |
| Zone 3                        | °C.   | Zone 3                  | 260     | 255     |
| Zone 4                        | °C.   | Zone 4                  | 260     | 255     |
| Melt Temperature              | °C.   |                         |         |         |

The poly(trimethylene terephthalate) BCF yarns and commercial nylon 6 and 66 yarns were tufted into 32 oz.  $\frac{5}{32}$  gauge cut-pile Saxony carpets having  $\frac{2}{32}$ " pile height. They were walk-tested with 20,000 footsteps accelerated floor trafficking for resiliency and appearance retention comparisons. Roll conditions and results are shown in Table 5.

55

The speed and temperature of the rolls, texturing conditions and yarn tensile properties are shown in Table 6. In Trial 1, the relax roll was a single roll with a follower, and in Trial 2, the relax roll was a dual roll. The spin finish was Goulston Lurol 3919 applied as a 25–30% emulsion. The first stage draw was about 1.13 (Trial 1) and 1.015 (trial 2) and second-stage draws were about 2.5 and 3.2. Although heat was not added to Roll 1 in these trials, the heat of operation would be expected to be above room temperature. As can be seen from Table 6, the yarn had excellent tenacity and elongation at speeds greater than 2000 m/min.

## EXAMPLE 7

Use of Low First-Stage Draw Ratio

Poly(trimethylene terephthalate) (0.9 i.v.) was spun into 69 filaments with trilobal cross-sections using a drawing and

TABLE 6

|                                  | Trial 1  | Trial 2  |
|----------------------------------|----------|----------|
| <u>Roll speeds (m/min.):</u>     |          |          |
| Roll 1                           | 430      | 754      |
| Roll 2                           | 486      | 765      |
| Dual Roll 3                      | 1226     | 2500     |
| Relax Roll                       | 1176     |          |
| Relax Dual Roll 4                |          | 2010     |
| Winder                           | 1156     | 1995     |
| <u>Roll Temperatures (° C.):</u> |          |          |
| Roll 1                           | Unheated | Unheated |
| Roll 2                           | 49       | 65       |
| Roll 3                           | 135      | 165      |
| Relax Dual Roll 4                | Unheated | Unheated |
| <u>Texturizing Conditions:</u>   |          |          |
| Air Jet Temperature (° C.)       | 163      | 190      |
| Air Jet Pressure (psi)           | 80       | 95       |
| Interlacer Pressure (psi)        | 20       | 30       |
| <u>Yarn Properties:</u>          |          |          |
| Yarn Count (denier)              | 1450     | 1328     |
| Tenacity (g/den)                 | 1.3      | 1.98     |
| Elongation (%)                   | 44       | 50.4     |

I claim:

1. A process for preparing bulk continuous fiber yarn from poly(trimethylene terephthalate) comprising:
  - (a) melt-spinning poly(trimethylene terephthalate) at a temperature within the range of about 250 to about 280° C. to produce a plurality of spun filaments;
  - (b) cooling the spun filaments;
  - (c) converging the spun filaments into a yarn;
  - (d) drawing the yarn at a first draw ratio within the range of about 1.01 to about 2 in a first drawing stage defined by at least one feed roller and at least one first draw roller, each of said at least one feed roller operated at a temperature less than about 100° C. and each of said at least one draw roller heated to a temperature greater than the temperature of said at least one feed roller and within the range of about 50 to about 150° C.;
  - (e) subsequently drawing the yarn at a second draw ratio of at least about 2.2 times that of the first draw ratio in

a second drawing stage defined by said at least one first draw roller and at least one second draw roller, each of said at least one second draw roller heated to a temperature greater than said at least one first draw roller and within the range of about 100 to about 200° C.; and

- (f) winding the drawn yarn.
2. The process of claim 1 which further comprises texturing the drawn yarn and cooling the textured filaments.
3. The process of claim 1 in which each of said at least one feed rollers is maintained at a temperature within the range of about 40 to about 85° C.
4. The process of claim 1 in which the first draw ratio is within the range of about 1.01 to about 1.35.
5. The process of claim 1 in which the second draw ratio is within the range of about 2.2 to about 3.4 times the first draw ratio.
6. The process of claim 1 in which the poly(trimethylene terephthalate) has an intrinsic viscosity within the range of about 0.80 to about 1.0 dl/g.
7. The process of claim 1 in which the poly(trimethylene terephthalate) has an intrinsic viscosity within the range of about 0.88 to about 0.96 dl/g.
8. The process of claim 1 in which the poly(trimethylene terephthalate) is the product of condensation polymerization of the reaction product of 1,3-propane diol and at least one of terephthalic acid and dimethyl terephthalate.
9. The process of claim 1 in which the poly(trimethylene terephthalate) is the product of condensation polymerization of the reaction product of (a) a mixture of 1,3-propane diol and a second alkane diol and (b) a mixture of terephthalic acid and isophthalic acid.
10. The process of claim 2 in which texturing is carried out with an air jet at a pressure within the range of about 50 to about 120 psi.
11. The process of claim 2 in which the product yarn bulk is within the range of about 15 to about 45 percent.
12. The process of claim 2 in which the yarn is fed to texturing via a feed roll maintained at a temperature within the range of about 150 to about 200° C.
13. The process of claim 2 in which the texturing step is carried out at a temperature within the range of about 150 to about 210° C.

\* \* \* \* \*